

Jan. 8, 1935.

A. E. VANDERCOOK

1,987,454

METAL SEPARATION

Filed March 6, 1934

2 Sheets-Sheet 1



Jan. 8, 1935.

A. E. VANDERCOOK

1,987,454

METAL SEPARATION

Filed March 6, 1934

2 Sheets-Sheet 2



## UNITED STATES PATENT OFFICE

1,987,454

## METAL SEPARATION

Albert E. Vandercrook, Sacramento, Calif., assignor  
to National Mining and Reduction Company,  
Sacramento, Calif., a corporation of California

Application March 6, 1934, Serial No. 714,349

15 Claims. (Cl. 75—185)

The invention relates to metal separation and particularly to the cyanide process of recovering precious metals such as gold.

Among the objects of the invention are: 1. to provide a direct flow decantation process wherein the pulp is not classified for separate treatment of the sand and slimes; 2. to shorten the time required for sending the major portion, as well as the whole, of the values to precipitation; 3. to obtain bullion free from matte or sulpho-compounds; 4. to discharge substantially all of the sulphides in the tailings, without using lead salts or other compounds requiring constant close supervision of the amount of such compound necessary; 5. to automatically generate or create in the solution the amount of compound necessary to pass substantially all of the sulphides, in insoluble form to the tailings; 6. to make the total recovery from the pregnant solution without effecting a portion of the recovery by amalgamation.

The important part that oxygen takes is facilitating the solution of gold in the lixiviating solution is well understood. It has heretofore been proposed to separately treat the sands and the slimes, allowing each to stand in its solution for a varying length of time up to several days, to permit the oxygen of the air to act on the solution. The prior process may be called the "batch" process, to distinguish it from the present process wherein the solution passes in a continuous manner through the apparatus in the same direction as the pulp, without separation of the sands and the slimes, whereby a considerable saving is effected, not only of time but also in the amount of water required.

It has heretofore been proposed to render the cyanide process continuous. According to pages 1043 to 1045 of the Hand Book of Metallurgy by Dr. Schnabel, published 1921, the only continuous process which has been used extensively is the Dorr continuous counter-current decantation process, which is generally employed as an all-slimering process in which the ore is crushed in cyanide solution. In that case, clear water and barren solution proceed through a series of thickeners in a direction opposite to the flow of the pulp there-through. The overflow from the first of the secondary thickeners is partly short circuited on itself through a series of agitators, the major portion being supplied to the tube mill and from thence to the primary thickener, the overflow from which goes to the precipitation

tank. Consequently, whatever values are recovered by the secondary thickeners, can only reach the precipitation tank by way of the primary thickener after passing through the tube mill. As distinguished from the Dorr process, my invention provides for the differential withdrawal of the pregnant solution from two separated points along the path of travel of the pulp solution, the first of these points being the overflow from the primary thickener (without previous recovery of amalgam and without previous agitation except that inherent in the ball mill and classifier) where concentrated pregnant solution is withdrawn to precipitation, and the second point being from one of the secondary thickeners, such as the first one, where the pulp has previously been subjected to agitation and to dilution from the barren solution resulting from precipitation. Also a part of the overflow from the selected one of the secondary thickeners and the overflow from a subsequent secondary thickener is regenerated to form aerated mercury cyanide solution which is returned to the ball mill. In this way, the values are returned quicker to precipitation, than heretofore. My process may be termed the direct flow decantation process to distinguish it from the counter-current process above mentioned.

My direct-flow continuous process is made possible, partly by the fact that the oxygen necessary to facilitate the chemical reaction is added to the solution by aeration, thereby avoiding the prolonged treatment heretofore required in the "batch" process.

The small usage of water, according to the present invention, results from the recovery of all of the solution except the small amount necessary to move out the pulp. Also in the final stages, the solution is diluted with fresh water and barren liquid from the precipitation system, whereby the cyanide and value loss is kept very low.

An important part of the invention resides in the chemistry of the recovery process. According to this feature of the invention, the ore in the ball mill is ground in the presence of mercury cyanide solution which has been aerated, hereafter called the solution, in order that the ore while being ground may be subjected to this solution. The important part that both mercury and oxygen have in this process are explained below.

Alkali cyanides in the presence of oxygen as

5

15

25

20

15

25

20

30

35

30

35

30

35

30

35

30

35

30

35

30

35

30

35

30

35

30

35

30

35

30

35

30

35

30

35

30

35

30

35

30

35

30

an oxidizer, dissolve mercury to form mercuric cyanide soluble in water and cyanides.



- 5 Mercury cyanide is soluble in eight parts of water at 15° C. It is also soluble in sodium and potassium cyanide solution. When sodium or potassium cyanide solutions, of the strengths used in metallurgical plants treating gold and 10 silver ores, is saturated with atomized air, mercury can be dissolved by the plant solutions.



It is conceded by most metallurgists that oxygen is indispensable for the solution of gold and silver from their ores by the ordinary cyanide 20 process solutions, and that it acts directly or indirectly.

In the mercury cyanide process, oxygen is absolutely necessary and performs three very important functions. First, as a depolarizer and an 25 oxidizer of mercury which oxide is being dissolved by sodium cyanide, also in the same manner while gold and silver are being dissolved from the ores.

Second, as an oxidizer of any reducing agents 30 that may start to form in the working solutions.

Third, as a most important oxidizing agent in gaseous form to replace all the reducing hydrogen gas released into the working solutions during the precipitation of the metals.

35 These three functions of oxygen are of the utmost importance.

The function of the mercury in mercury cyanide solutions is five-fold.

First, as a disintegrator of the gold particles. 40 It is easily proven that gold obtained from panning ore when mercury cyanide solution is added is immediately coated with mercury and starts to disintegrate the particles of gold.

Second, as an assisting agent for the more 45 rapid solution of gold and silver in their ores. This has been repeatedly proven in comparative tests in the laboratory and in actual plant operation.

Third, as a precipitant for alkaline sulphides 50 that start to form in the working solutions of a plant. Mercury has a greater affinity for sulphur than for cyanide and forms with sulphur insoluble HgS and so keeps the working solutions from becoming foul with interfering elements.

Fourth, improve fineness of bullion recovered 55 by keeping sulphids and other base metals out of precipitate.

Fifth, economy due to eliminating necessity for adjunctive chemicals, and to small amount 60 of mercury itself which is required.

The action of mercuric salts in cyanidation is well known. However added, mercuric chloride, or otherwise, mercury in cyanide solution probably functions as the compound— $\text{K}_2\text{Hg}(\text{CN})_4$ . 65 The chemistry of this salt is well known, and it functions in solution of gold and silver without the intervention of oxygen. The innovation in my invention is not in the use of any mercury salts, but in the method of its formation and introduction into the cyanide solution; that is, the use of mercury in the cycle in metallic form and the dissolving thereof in alkali cyanide to form the desired double cyanide. This reaction, I have established. In the passage of the usual working 70 mill solution of alkali through a mercury cyanide

generator, a small amount of mercury is dissolved and is present in all of my working solutions at all times.

Oxygen is necessary for this solution effect, and the amount dissolved can be controlled by introducing or excluding a regulated amount of dissolved oxygen. While, as stated above, dissolved mercury is present in all my solutions, the amount dissolved is never great; for only rarely are even traces of mercury found upon 10 the zinc shavings or zinc dust in precipitation. The usual amount found to be present in solution is of the order of .01% to .015% and less.

This solvent action of alkali mercury cyanide is a very efficient aid in extraction, particularly 15 upon some of the more difficult soluble silver minerals, and it has been found materially to shorten the time of treatment of complex gold ores.

Another function of dissolved mercury in solution is that for which salts of lead are usually 20 employed, viz., the removal of "soluble" sulphide sulphur by the precipitation of the very insoluble mercuric sulphide. The use of lead salts in cyanidation is usually haphazard and most difficult of intelligent control. In my system, mercury is always present in our solutions and a 25 regulated amount of aerated mercury cyanide is formed automatically as needed.

In the development of this process and system, 30 opportunity was offered to overcome many difficulties found in usual cyanide practice and this resulted in most cases in complete extraction during crushing, instead of long agitation, thereby shortening the time cycle. Heating of solutions as with silver ores is not required.

*The solubility and effect of metallic mercury in cyanide solutions*

First. A .25% or 5 lb. solution of potassium cyanide was left in contact with mercury in agitation with free access of air to the surface for 40 15 hours, and showed a solubility of mercury equal to .019%. A .3% or 6 lb. solution of sodium cyanide was similarly treated and gave mercury .022% in solution.

These simple experiments were merely qualitative, other factors such as temperature, dissolved oxygen were not taken under control.

The solubility in some cases, is affected by difference of concentration and temperature 50  $\text{Hg} + 4\text{KCN} + \text{H}_2\text{O} + \text{O} = \text{K}_2\text{Hg}(\text{CN})_4 + 2\text{KOH}$ . This is analogous to the "Elsner's Equation" for gold and silver. Julian and Smart give  $\text{Hg} + 4\text{KCN} + 2\text{H}_2\text{O} = \text{K}_2\text{Hg}(\text{CN})_4 + 2\text{KOH} + \text{H}_2$ . Preference is for the former statement of the reaction—in either case oxygen is essential, either entering directly into the reaction or as combining with evolved hydrogen, removing it from occlusion so that the reaction may proceed.

The necessity for dissolved oxygen cannot be 60 too strongly emphasized. The amount of mercury going into solution in a given time is directly controlled by the amount of oxygen available and the oxygen derived from pure water has no significance when one considers conditions met in ordinary practice. The effect of the dissolved salts and solids in suspension by increasing viscosity and by chemical reactions, decrease the solubility of oxygen, and these factors vary 65 enormously in practice. Consequently, the amount of mercury going into solution under working conditions is slight.

Second. Desulphurizing action of mercury in solution:—The reaction whereby the sulphur of 70 sulfide minerals of ores enter into solution in 75

working solutions are obscure and exceedingly complicated, although the deleterious effect of alkali sulfides is well known, they are powerful reducing agents and cyanicides.  $K_2S + KCn + H_2O + O = KCnS + 2KOH$ ; also they precipitate dissolved silver as silver sulfides and may under certain conditions precipitate gold and silver. In ordinary practice, soluble lead salts are added to remove alkali sulfides, by the precipitation of lead sulfides. This practice is not subject to exact control, and is governed usually by guess. Mercury salts are equally effective as lead salts.



My solution has an efficient desulphurizing action at the moment of formation of alkali sulfides, with advantages over former practice.

Third. Dissolving power of mercuric cyanide  $K_2Hg(CN)_4$  on gold and silver.

This effect is well established, and takes place without the intervention of oxygen.



In practice it is probably more marked as an aid in the dissolving of silver.

In the non-continuous cyanide process in common use, in spite of the recognized advantages of recovering the coarser metallic particles of gold and silver, upon which the dissolving effect of cyanide is slow, when crushing in solution, amalgamation is not largely practised. There is always a mechanical loss of mercury and of amalgam from the plates which finds its way in part into the tails. In my system such loss is impossible, as the coarse or heavy gold or silver particles remain in the grinding circuit until dissolved.

Another and more serious disadvantage in the noncontinuous cyanide process in common use is the presence of metallic copper. The deleterious action of copper on cyanide is well known, a source of loss from beginning to end by consumption of cyanide, by deterioration and solution of plates by reducing action, (loss of oxygen), by consumption of zinc, by introduction of copper into precipitates and bullion. In this system the use of copper as metal or alloy is entirely avoided.

Mercury not so consumed by alkaline sulfides is free to aid as a solvent, while lead salts have no such action and are rather deleterious than otherwise. The necessary and uncertain excess of lead salts tend to be lost as sulphate or carbonate, serving no useful purpose.

No mercury is found on the zincs under normal working conditions. The mercuric cyanide  $K_2Hg(CN)_4$  performs its functions as formed and does not accumulate in the solutions. The consumption of mercury is light and the cost per ton insignificant as only 5 to 7 lbs. is required for 25,000 tons of ore treated.

The above described solution reaction throughout the cycle has rendered bullion free from matte or sulpho compound. The precipitate requires no preliminary treatment, such as an acid treatment, and can be fluxed and melted direct into bullion.

The presence of mercury in the solution is also beneficial in assisting the precipitation of the precious metals.

In carrying out the invention, the various pieces of apparatus employed in the recovery

process are arranged approximately in a circular array, with a pilot house in the center thereof, the various pieces of apparatus being arranged for the most part at a level equal to or less than the level of the pilot house, whereby a single operator in the pilot house can watch substantially all of the pieces of apparatus in operation. Furthermore, remote control switches for operating the various motors in the system, together with indicators for indicating the height of the liquid in a stock tank or other tanks, are all brought together on a common switchboard at a convenient point in or adjacent the pilot house, thereby further facilitating the control of the apparatus by a single operator. The use of this continuous process, with the convenient arrangement of apparatus above described, makes it possible for a single operator to run a mill handling 150 tons or more of ore per day.

I have discovered that a major portion of recovery, viz. 90%, is had by the time the pulp leaves the classifier and I immediately decant or thicken the pulp and pass the pregnant solution to precipitation. A further advantage of not agitating prior to the first thickening is to avoid emulsifying any carbon present, as with my arrangement the carbon floats on the surface of the first thickener and can be removed by skimming.

For further details of the invention reference may be made to the drawings, wherein:

Fig. 1 is a flow diagram somewhat in vertical aspect, the path of the pulp being indicated by dashed lines.

Fig. 2 is a flow diagram, in horizontal aspect, indicating the general arrangement of the apparatus around the pilot house.

Referring to Fig. 1, the ore from a car is dumped on grizzly 1, the ore passing through the grizzly being received by a belt conveyor 2, the ore retained by the grizzly being supplied to a gyratory crusher 3 which delivers crushed ore to the belt 2 as will be readily understood. Lime is added to the crushed ore on belt 2 from the container 4. The belt 2 delivers the mixture of lime and crushed ore to the ball mill 5, to both the heads and the tails of which are continuously supplied the solution, i. e. aerated mercury cyanide solution, from a stock tank 6. A launder 8, if desired, may contain riffles to catch large particles of gold or silver and retain the same until they are removed or finally dissolved by the solution, instead of returning them to the ball mill.

The output from the ball mill 5 is supplied to a Dorr classifier 7 which returns the sands to be reground by the ball mill 5, the pulp, that is slimes, or sand and slimes which have been ground to a suitable fineness are supplied by gravity through the launder 9 to the number 1 primary thickener.

Pulp from the bottom of primary thickener number 1 is pumped by diaphragm pump 10 to the top of agitator 11. Pulp from the top of agitator 11 flows by gravity to the top of agitator 12. Pulp from the top of agitator 12 flows to the top of secondary thickener number 2 and from the bottom of latter pulp is pumped by diaphragm pump 13 to the top of another secondary thickener number 3. From the bottom of thickener number 3 pulp is pumped by diaphragm pump 14 to the tailings discharge 15.

The pregnant solution flows by gravity from thickener number 1 to the clarifying filter 16 to which is also supplied pregnant solution from 75

the thickener number 2. The filter 16 clarifies the overflow solution from the thickeners number 1 and number 2, removing for example talc. The filter 16 may be of the well known leaf type.

This prepares the solution for the precipitation of gold and silver by zinc dust or the like. The clarified solution is drawn from filter 16 by pump 17 which discharges to an indicator tank 18, the 10 discharge from the latter being pumped by a vacuum pump 19 and then by gravity to a zinc dust emulsifier 20. The emulsifier 20 supplies in parallel a large number of collecting bags indicated at 21. The barren liquid from the precipitation or collecting bags 21 flows by gravity to a device which forms an important part of this invention and which I have termed a mercury generator, indicated at 22, to receive the barren liquid from bags 21 and also indicated at 23 to 15 receive the overflow from thickeners number 2 and number 3. This mercury generator is of the construction shown in my Patent No. 1,156,946 and comprises a tank 24 having rotatably mounted therein a rotatable pipe 25 having oppositely extending discharge nozzles 26 and 27 communicating with the axial pipe 28 which receives the discharge from the pump 29, the inlet to this pump being taken from the bottom of the tank 22. Air is admitted to the inlet of pump 29 by the valve 30, to aerate the solution. The discharge from pump 29 through the nozzles 26 and 27 causes the arm 25 carrying these nozzles to rotate and distribute the discharged liquid over the surface of a pool of mercury 31 in the bottom of the 35 tank 22, to thereby form aerated mercury cyanide solution.

According to my prior patent above mentioned, and also according to my Patent No. 1,135,080, I proposed to supply to the mercury generator the 40 solution together with sand and slimes, whereas according to the present invention the mercury generator operates only on clear solution from which the sand and slimes have been removed.

Furthermore, according to the present invention 45 the mercury generator is to better advantage connected into the system at points other than the points disclosed in my previous patents.

In accordance with the chemistry heretofore explained, it will be understood that generators 50 22 and 23 serve as sources of aerated mercury cyanide solution. The output from the mercury generator 22 discharges partly at the pulp input to agitator 11 and partly at the pulp input to agitator 12, to dilute the solution at these points 55 and to subject the same to the benefit of the aerated mercury cyanide solution as heretofore explained.

The mercury generator 23 receives the overflow from thickeners number 2 and number 3 and furnishes aerated mercury cyanide solution to the sump 32 from which it is drawn by pump 33 to the stock tank 6, in order that the ore in the ball mill 5 at the very outset may be treated 60 with aerated mercury cyanide solution with the 65 benefits before mentioned.

Solution is supplied to the mercury generators 22 and 23, from precipitation, and from the thickeners numbers 2 and 3 respectively, at the 70 return of about 60 gallons per minute. The area of the mercury surface in each of the generators 22 and 23 is about 700 square inches. The area of the air inlet controlled by valves 30 and 38 is about one-eighth inch in diameter. The speed of the pump 29 and of the corresponding pump 75 for generator 23 is about 1200 R. P. M. The

amount of air drawn in can be controlled by regulating the valves 36 and 37 in the inlet to the pumps such as 29. The relation of the elements is such that there is a fraction of 1%, such as .01% to .015% and less of mercury in all parts of the system.

Fresh water from a pipe 34 is supplied to the outlet of pump 13 in order to replace the small amount of water required to move the tailings to the discharge 15, and to further dilute the solution carrying the pulp, the initial dilution being obtained in the agitators 11 and 12 by the barren liquid from the generator 22, as above explained. Also, from time to time, sodium cyanide is added to the system, for instance in generator 23, to 15 replace the cyanide lost in the tails. Safety or overflow pipe lines 39, 40, 41, and 42 are provided as indicated.

A plan view of the apparatus is indicated in Fig. 2. Except for the stock tank 6, which is elevated, and except for the sump 32 in the basement of the mill, the various pieces of apparatus are arranged generally at the level of pilot house 35 which is centrally located with respect thereto. Remote control switches for the motors driving 20 the various pumps and for the motor driving the ball mill 5, as well as indicators showing the level of the liquid in the tanks 6 and 17, are brought to a common point in or on the pilot house, whereby a single operator may readily control 25 all of the apparatus. The pilot house is completely surrounded with glass windows to keep out the noise of the mill while permitting the attendant to inspect all of the apparatus from a central point within the pilot house.

Practical experience with the process herein disclosed has shown that a recovery of the order of 97% in gold can be made from low grade ore assaying from \$5.00 to \$7.00 per ton, while handling 100 tons per day. The strength of the cyanide solution used in the stock tank is about 1.1 lb. per ton of solution. The time of the cycle is 9½ hours. The ore is ground so that about 97% is -100 mesh and about 75% is -200 mesh. The consumption of sodium cyanide is about ½ pound per ton of ore including tailing loss and the consumption of zinc dust about .025 pound per ton of ore treated.

For the first three weeks this mill was in operation, the values in the bags plus the tailing loss was approximately two-thirds the value of the mill heads, showing, as was later verified by results, that coarse gold not readily soluble, was remaining in the grinding circuit. It was not until twenty one days after starting the mill that the recovery plus the tailings loss was as large as the values in the mill heads. In fact, after the three weeks' period had elapsed, the recovery in the bags was frequently higher than the value of the mill heads, so that the average results over operations for 6 or 8 weeks checked out properly. The recovery therefore is preferably made wholly from the pregnant solution without attempting to recover the coarse gold by amalgamation on a copper plate as the latter has disadvantages pointed out above.

It will be apparent that various modifications may be made in the process and apparatus herein disclosed without departing from the spirit of the invention.

Having thus described the invention, what is claimed as new and desired to secure by Letters Patent is:

I claim:

1. The steps in the method of metal separation which comprises grinding ore in the presence of aerated mercury cyanide solution, forming said mercury cyanide solution by aeration of cyanide solution in the presence of metallic mercury, and in controlling the amount of aeration to control the amount of mercury in solution whereby the sulphids present in the pulp pass substantially wholly into the tailings, and recovering the values in solution substantially wholly by lixiviation. 5
2. The steps in the method of metal separation which comprises classifying wet pulp in the presence of aerated mercury cyanide solution, forming said mercury cyanide solution by aeration of cyanide solution in the presence of metallic mercury, and in controlling the amount of aeration to control the amount of mercury in solution whereby the sulphids present in the pulp pass substantially wholly into the tailings, and recovering the values in solution substantially wholly by lixiviation. 10
3. The steps in the method of metal separation which comprises agitating wet pulp in the presence of aerated mercury cyanide solution, forming said mercury cyanide solution by aeration of solution substantially free from pulp, and in controlling the amount of aeration whereby the sulphids present in the pulp pass substantially wholly into the tailings, and recovering the values in solution substantially wholly by lixiviation. 15
4. Improvement in the cyanide process of metal separation which comprises grinding ore in the presence of aerated mercury cyanide solution, directly separating the ground ore from the pregnant solution without previous agitation after grinding, treating the pregnant solution to recover the metal dissolved therein, aerating the resulting barren solution in the presence of mercury to form aerated mercury cyanide solution and in subjecting the ground ore to the last mentioned solution. 20
5. The continuous cyanide process of metal separation which comprises grinding ore in the presence of a continuous supply of aerated mercury cyanide solution, continuously thickening and then agitating the resulting pulp, continuously removing clear pregnant solution from the pulp thus treated and precipitating metal therefrom, continuously passing the tailings, with sand and slimes together, to a tailings dump, returning the barren liquid resulting from said precipitation, to increase the fluid content of the pulp solution after initial thickening, adding enough fresh water to replace the fluid required to move the tailings to a point of discharge and to further reduce dissolved values in the thickened pulp, and regenerating the overflow from said thickening to provide said aerated mercury cyanide solution in the presence of which said ore is ground. 25
6. Improvement in the cyanide process of metal separation which comprises grinding ore in the presence of aerated mercury cyanide solution, decanting pregnant solution therefrom, precipitating metal from said pregnant solution to form barren solution, diluting pulp resulting from said decantation with said barren solution to form diluted pregnant solution, decanting said diluted pregnant solution partly for said precipitation and partly for the formation of aerated mercury cyanide solution, treating the decanted liquid to form said aerated mercury cyanide solution and supplying said aerated mercury cyanide solution for said grinding. 30
7. Metal separation apparatus comprising the combination of means for supplying pulp in cyanide solution, an agitator therefor, means for decanting clear liquid from said pulp, an aerated mercury cyanide generator, means for supplying said clear liquid to said generator, said generator comprising a tank, a pool of mercury in said tank, a pump for aerating the liquid in said tank and returning the same over said pool of mercury, means for withdrawing aerated mercury cyanide solution from said tank and for adding the same to the pulp supplied to said agitator. 35
8. Metal separation apparatus comprising the combination of a precipitation unit, an aerated mercury cyanide generator, an agitator, means for supplying filtrate from said precipitation unit to said generator, and means for supplying aerated mercury cyanide solution from said generator to said agitator. 40
9. Metal separation apparatus comprising the combination of a plurality of thickeners, a precipitation unit, an aerated mercury cyanide generator, means for supplying overflow from said first of said thickeners partly to said precipitation unit and partly to said generator, means for supplying overflow from said second thickener to said generator, means for diluting with fresh water the pulp from said second thickener, and a sump tank in circuit with said generator. 45
10. Improvement in the cyanide process of metal separation which comprises grinding ore in the presence of aerated mercury cyanide solution, successively thickening, agitating, and thickening the pulp and thereafter again thickening the pulp, said last mentioned thickening being in the presence of fresh water, and thereafter passing the pulp to a tailings discharge, withdrawing the overflow from said first mentioned and second mentioned thickening for precipitation of the metal, passing the resulting barren solution to dilute the pulp at said point of agitation, and aerating the overflow from said third mentioned thickening in the presence of mercury to form the aerated mercury cyanide solution in the presence of which the ore is ground. 50
11. Process according to claim 10 wherein said barren solution is aerated. 55
12. Process according to claim 10 wherein said barren solution and the overflow from said third mentioned thickening are aerated in the presence of mercury to form aerated mercury cyanide solution. 60
13. The direct flow decantation cyanide process of metal separation which comprises grinding ore in the presence of aerated mercury cyanide solution, decanting the pregnant solution from the pulp, precipitating the metal from the pregnant solution, aerating the barren solution in the presence of mercury, mixing the pulp with said last mentioned solution and thereafter subjecting the same to agitation and decantation, and aerating in the presence of mercury the overflow from said last mentioned decantation to provide the solution for said grinding. 65
14. The steps in the method of metal separation which comprises aerating cyanide solution substantially free from pulp in the presence of metallic mercury to form mercury cyanide which is soluble in cyanide solution, said aeration also being carried out to a point to provide an excess of oxygen which facilitates the solution of precious metal or metals in the cyanide solution, controlling the amount of said aeration to control the amount of the compound of mercury which is formed in solution, whereby sulphides 70
- 75

which would otherwise be soluble are prevented from going into the solution due to the presence of mercury in said solution, said sulphides therefore passing in solid form substantially wholly into the tailings, and recovering the values substantially wholly by lixiviation in said solution without substantial recovery by amalgamation.

15. Metal separation apparatus comprising the combination of apparatus for dissolving metal in and recovering metal from cyanide solution, and means in circuit therewith for continuously generating aerated mercury cyanide solution from cyanide solution substantially free from pulp. 5

ALBERT E. VANDERCOOK.